

# United States Patent [19]

Degueldre et al.

[11] 3,849,282

[45] Nov. 19, 1974

[54] METAL ELECTRODES AND COATINGS  
THEREFOR

[75] Inventors: Louis Degueldre; Charles Killens;  
Louis Bourgeois, all of Brussels,  
Belgium

[73] Assignee: Solvay & Cie, Brussels, Belgium

[22] Filed: July 3, 1972

[21] Appl. No.: 268,552

[30] Foreign Application Priority Data

July 9, 1971 Luxembourg ..... 63506

[52] U.S. Cl. .... 204/290 F, 204/290 R, 204/291

[51] Int. Cl. .... B01k 3/06

[58] Field of Search ..... 204/290 F, 290 R, 291

[56] References Cited

UNITED STATES PATENTS

3,491,014 1/1970 Bianchi et al. .... 204/242

|           |         |                  |           |
|-----------|---------|------------------|-----------|
| 3,562,008 | 2/1971  | Martinsons ..... | 117/221   |
| 3,632,498 | 1/1972  | Beer .....       | 204/290 F |
| 3,701,724 | 10/1972 | Entwistle .....  | 204/290 F |

Primary Examiner—F. C. Edmundson  
Attorney, Agent, or Firm—Spencer & Kaye

[57] ABSTRACT

Conductive coating for metal electrodes, consisting essentially of a compound  $ABO_4$  with a structure of the rutile-type, where A represents an element in the trivalent state selected from the group consisting of Rh, Al, Ga, La, and the rare earths and B represents an element in the pentavalent state selected from the group consisting of Sb, Nb and Ta, and an oxide of the type  $MO_2$  where M is selected from the group consisting of Ru and Ir.

5 Claims, No Drawings

## METAL ELECTRODES AND COATINGS THEREFOR

### BACKGROUND OF THE INVENTION

The present invention relates to a new type of coating intended for constituting the active surface of a metal electrode made at least superficially of titanium or a titanium alloy and optionally containing a core of a better conducting material than titanium, for example of copper, aluminum, iron or alloys of these metals.

Electrodes provided with a coating having catalytic properties according to the present invention may be used in various electrochemical processes such as cathodic protection, desalination or purification of water, electrolysis of water or hydrochloric acid, production of current in a fuel cell, reduction or oxidation of organic compounds of the electrolytic manufacture of per salts, but they are particularly useful as anodes in the electrolysis of aqueous solutions of alkali metal halides, particularly sodium chloride, both in diaphragm cells and mercury cells where they catalyze the discharge of chloride ions which is brought about at a remarkably low and practically constant overpotential throughout the whole life of the electrode. Under the conditions ruling in these cells, wear of the coating is insignificant, and this assures a practically unlimited life for the anodes and avoids the burdensome operations of opening the cells and renewing the coatings.

### SUMMARY OF THE INVENTION

An object of the present invention, therefore, is to provide an electrocatalytically active coating which is particularly well adherent to its metallic support and is resistant to electrochemical corrosion.

This as well as other objects which will be apparent are achieved by a new type of coating for metal electrodes, which coating comprises a compound  $ABO_4$  having a rutile-type structure, where A is an element in the trivalent state selected from the group rhodium, aluminum, gallium, lanthanum and the rare earths, while B is an element in the pentavalent state selected from the group antimony, niobium and tantalum, the compound  $ABO_4$  being associated with an oxide of the type  $MO_2$  where M is ruthenium and/or iridium.

### DESCRIPTION OF THE PREFERRED EMBODIMENTS

The molecular ratio  $ABO_4/MO_2$  is preferably between 1/1 and 1/6.

It is preferred to place the conductive coating of the present invention on a metal support at least superficially made of titanium or a metal of titanium group. Advantageously, titanium is clad on a core of a more conductive metal such as copper, aluminum, iron, or alloys of these metals.

Preferably, the coating of the present invention consists essentially of the compounds as defined in the SUMMARY OF THE INVENTION; yet more preferably, the coating consists of those compounds.

The compounds  $ABO_4$  and  $MO_2$  must be present together in the coating. It may be possible to maintain the  $ABO_4/MO_2$  mol ratio in a wide range for several electrochemical processes.

However, it has been found advantageous to maintain this ratio between well defined limits when the conductive coating is intended for the manufacture of

metallic anodes for the electrolysis of aqueous solutions of alkali metal halides, especially sodium chloride. If the proportion of  $MO_2$  is too low, the overvoltage is higher than 300 mV (measured according to test of Example 1) and if the proportion of  $MO_2$  is too high, the consumption of noble metal/ton of produced chlorine is prohibitive, i.e., higher than 40 mg/t  $Cl_2$ . For these reasons, the  $ABO_4/MO_2$  mol ratio is maintained between 1/1 and 1/6.

Among all the elements for A in the trivalent state, Rh and Al have always given better results, so they are preferred.

Further illustrative of the present invention are the following Examples:

15 Example 1 :  $ABO_4 \cdot 2MO_2$  where A = Rh, B = Sb and M = Ru

A solution A containing 0.5 g-atom ruthenium/liter was prepared by dissolving ruthenium trichloride ( $RuCl_3 \cdot xH_2O$ ) in n-hexanol, a solution B containing 0.5 g-atom rhodium/liter was prepared by dissolving rhodium trichloride ( $RhCl_3 \cdot xH_2O$ ) in n-hexanol and a solution C containing 1 g-atom antimony/liter was prepared by dissolving antimony pentachloride ( $SbCl_5$ ) in n-hexanol.

20 25 By mixing 6.6 ml of solution A, 3.3 ml of solution B, 1.6 ml of solution C and 38.5 ml of n-hexanol, there was obtained a composition which was applied in 7 layers onto plates of titanium that had previously been hot-degreased in trichloroethylene and etched for, 5 hours at approximately 90°C in an aqueous solution of oxalic acid containing 100 g/liter. For application of this composition, the titanium plates were placed in air on a hotplate at a temperature of about 75°C.

30 35 After each application the plates were dried and then heated for 15 minutes at 500°C and, after the 7th application, heated for 1 hour at 500°C, in the presence of air.

The amount of material thus deposited was approximately 4.5 g/m<sup>2</sup>.

40 45 The coating, which contained 2 g-atom Ru to 1 g-atom Rh and 1 g-atom Sb, showed excellent adherence to the substrate, as was shown in stripping tests with adhesive tape applied by pressure.

The plates of titanium thus coated were submitted to two types of evaluation.

The first relates to the over-potential for liberation of chlorine. It is measured at an anodic current density of 10 kA/m<sup>2</sup>.

50 55 The second relates to the consumption of noble metal as a function of the amount of chlorine liberated.

The measurement of over-potential is carried out by immersing the plates in brine containing 250 g NaCl/kg, saturated with chlorine at 60°C and at a pH of approximately 2. Under these conditions, the plates referred to in this example show an initial overpotential of approximately 165 mV and then an overpotential of 210 mV and 248 mV after a production of 67 and 210 tons of chlorine/m<sup>2</sup> respectively, while positively polarized under a current density of 10 kA/m<sup>2</sup>.

In another test the consumption of noble metal from these plates was evaluated by using them as anodes in a cell with a flowing mercury cathode containing brine saturated with chlorine and sodium chloride at a temperature between 80° and 85°C with a constant anode-cathode potential. Under these conditions the plates tested have already produced more than 264 tons of

chlorine/m<sup>2</sup>, at this time the limit of the useful life of the electrode had not yet been reached and the consumption test was continued, but it was already apparent that the consumption of noble metal would be less than 10 mg/ton of chlorine produced.

It was noted that the same plates showed an over-potential of approximately 210 mV at 10 kA/m<sup>2</sup> after producing approximately 67 tons of chlorine/m<sup>2</sup>.

Example 2: ABO<sub>2</sub>.2MO<sub>2</sub> where A = Rh, B = Nb and M = Ru

To 6 ml of solution A of Example 1 were added 3 ml of solution B of Example 1, 1.5 ml of a solution D containing 1 g-atom niobium/liter obtained by dissolving niobium pentachloride (NbCl<sub>5</sub>) in n-hexanol, and 39.5 ml of n-hexanol.

Ten layers of this composition were applied to plates of titanium etched as in Example 1. The various heat treatments were carried out in the same manner.

The average weight of the coating thus obtained was approximately 3.7 g/m<sup>2</sup>; it contained 2 g-atom Ru to 1 g-atom Rh and 1 g-atom Nb. The adherence to the substrate was very good. When used as anodes under the conditions specified in Example 1, the plates thus coated showed over-potentials of approximately 245 mV at an anodic current density of 10 kA/m<sup>2</sup>. During the consumption test carried out as in Example 1, the amount of chlorine already produced was 81 tons/m<sup>2</sup>, which corresponds to a consumption of noble metal equal to 26 mg/ton of chlorine.

Example 3: ABO<sub>4</sub>.2MO<sub>2</sub> where A = Al, B = Sb and M = Ru

A solution E containing 1 g-atom aluminum/liter was prepared by dissolving aluminum trichloride (AlCl<sub>3</sub>) in n-butanol.

To 10 ml of solution A of Example 1 were added 2.5 ml of solution C of Example 1, 2.5 ml of solution E and 35.0 ml of n-hexanol.

The application of this composition, in 8 coats, to 4 plates of etched titanium, and the heat treatments were carried out as in Example 1. The average weight of the coatings thus obtained was approximately 6 g/m<sup>2</sup>; they contained 2 g-atom Ru to 1 g-atom Al and 1 g-atom Sb. The adherence to the substrate was excellent.

When used as anodes under the conditions defined in Example 1, the plates thus coated showed an initial over-potential of 156 mV at an anodic current density of 10 kA/m<sup>2</sup>.

During the consumption test carried out as in Example 1, the amount of chlorine already produced was 125 tons/m<sup>2</sup>, which corresponds to a consumption of noble metal equal to 20 mg/ton of chlorine.

Example 4: ABO<sub>4</sub>.2MO<sub>2</sub> where A = Rh, B = Sb and M = Ir

To 2.8 ml of a solution F containing 1 g-atom of iridium/liter obtained by dissolving chloroiridic acid (H<sub>2</sub>IrCl<sub>6</sub>.xH<sub>2</sub>O) in n-hexanol were added 2.8 ml of solution B of Example 1, 1.4 ml of solution C of Example 1 and 43.0 ml of n-hexanol.

The application of this composition, in 10 coats, to plates of etched titanium and the heat treatments were carried out as in Example 1. The weight of the coatings thus obtained was approximately 6 g/m<sup>2</sup>; they contained 2 g-atom Ir to 1 g-atom Rh and 1 g-atom Sb. The adherence to the substrate was excellent.

When used as anodes under the conditions defined in Example 1, the plates thus coated showed initial over-

potentials of approximately 200 mV at an anodic current density of 10 kA/m<sup>2</sup>.

When submitted to the consumption test under the same conditions as in Example 1, the plates had produced more than 172 tons of chlorine/m<sup>2</sup>. At this time, the limit of useful life of the electrode had not yet been reached and the consumption test was continued, but it was already apparent that the consumption of noble metal would be less than 23 mg/ton of chlorine produced.

Example 5: ABO<sub>4</sub>.4MO<sub>2</sub> where A = Rh, B = Sb and M = Ir

To 1.6 ml of the solution F of Example 4 there were added 0.8 ml of solution B of Example 1, 0.4 ml of solution C of Example 1 and 47.2 ml of n-hexanol.

The application of this composition, in 10 coats, on plates of etched titanium and the thermal treatments were carried out as in Example 1.

The weight of the coatings thus obtained was approximately 3 g/m<sup>2</sup>; they contained 4 g-atom Ir to 1 g-atom Rh and 1 g-atom Sb. The adherence to the substrate was excellent.

When used as anodes under the conditions specified in Example 1, the plates thus coated showed over-potentials of approximately 230 mV at an anodic current density of 10 kA/m<sup>2</sup>.

When submitted to the consumption test under the same conditions as in Example 1, the plates had produced more than 198 tons of chlorine/m<sup>2</sup>. At this time, the limit of useful life of the electrode had not yet been reached and the consumption test was continued, but it was already apparent that the consumption of noble metal would be less than 11 mg/ton of chlorine produced.

Example 6: ABO<sub>4</sub>.2MO<sub>2</sub> where A = Rh, B = Sb and M = ⅔ Ru + ⅓ Ir

To 5.5 ml of the solution A of Example 1 there were added 1.4 ml of the solution F of Example 4, 4.2 ml of the solution B of Example 1, 2.1 ml of the solution C of Example 1 and 36.8 ml of n-hexanol.

The application of this composition, in 8 coats, to plates of etched titanium and the thermal treatments were carried out as in Example 1.

The weight of the coatings thus obtained was approximately 7 g/m<sup>2</sup>; they contained 4 g-atom Ru to 2 g-atom Ir, 3 g-atom Rh and 3 g-atom Sb; the adherence to the substrate was excellent.

When used as anodes under the conditions specified in Example 1, they showed an initial over-potential of approximately 135 mV and then at 202 mV after the liberation of 233 tons/m<sup>2</sup> of chlorine, at an anodic current density of 10 kA/m<sup>2</sup>. At this time, the limit of useful life of the electrode had not been reached and the consumption test was continued, but it was already apparent that the consumption of noble metal would be less than 18 mg/ton of chlorine produced.

Example 7: ABO<sub>4</sub>.2MO<sub>2</sub> where A = Rh, B = Sb and M = ⅔ Ru + ⅓ Ir

To 2.1 ml of the solution A of Example 1 there were added 2.1 ml of the solution F of Example 4, 3.2 ml of the solution B of Example 1, 1.6 ml of the solution C of g-atom Ir 1 and 41.0 ml of n-hexanol.

The application of the composition, in 8 coats, to plates of etched titanium and the heat treatments were carried out as in Example 1.

The weight of the coatings thus obtained was approximately 6 g/m<sup>2</sup>; they contained 2 g-atom Ru to 4 g-atom

Ir, 3 g-atom Rh and 3 g-atom Sb; the adherence to the substrate was excellent.

When used as anodes under the conditions specified in Example 1, the plates thus coated showed an initial overpotential of approximately 135 mV and then of 172 mV after the liberation of 150 tons of chlorine/m<sup>2</sup>.

After production of 225 tons of chlorine/m<sup>2</sup>, the limit of useful life of the electrode had not yet been reached and the consumption test was continued, but it was already apparent that the consumption of noble metal would be less than 17 mg/ton of chlorine produced.

Example 8:  $ABO_4.2MO_2$  where A = Rh, B = Sb and M = Ru

To 15.2 ml of the solution A of Example 1, there were added 7.6 ml of the solution B of Example 1, 3.8 ml of the solution C of Example 1 and 23.4 ml of n-hexanol.

The application of the composition, in 8 coats, to plates of etched titanium and the heat treatments were carried out as in Example 1.

The average weight of the coatings thus obtained was approximately 12.0 g/m<sup>2</sup>; they contained 2 g-atom Ru to 1 g-atom Rh and 1 g-atom Sb. The adherence to the substrate was very good.

When used as anodes under the conditions specified in Example 1, the plates thus coated showed an initial overvoltage of approximately 112 mV and then of 160 mV after the liberation of 225 tons of chlorine/m<sup>2</sup> of anodic surface at an anodic current density of 10 kA/m<sup>2</sup>. At this time, the limit of useful life of the electrode had not yet been reached and the consumption test was continued, but it was already apparent that the consumption of noble metal would be less than 29 mg/ton of chlorine produced.

Example 9:  $ABO_4.4MO_2$  where A = Rh, B = Ta and M = Ru

A solution G containing 0.5 g-atom/liter was prepared by dissolving ruthenium trichloride  $RuCl_3 \cdot xH_2O$  in isopropanol, a solution H containing 0.5 g-atom/liter by dissolving rhodium trichloride  $RhCl_3 \cdot xH_2O$  in isopropanol and a solution I containing 1 g-atom Ta/liter by dissolving tantalum pentachloride  $TaCl_5$  in methanol.

By mixing 8 ml of solution G, 2 ml of solution H, 1 ml of solution I and 39 ml of isopropanol, a coating composition was obtained, which was applied, in 10 coats, to plates of titanium etched under the same conditions as in Example 1. After each application, the plates were dried and heated for 15 minutes at 500°C, and after the tenth application, heated for 2 hours at 500°C in the presence of air.

The average weight of the coatings thus obtained was approximately 9.9 g/m<sup>2</sup>; they contained 2 g-atom Ru to 1 g-atom Rh and 1 g-atom Ta. The adherence to the substrate was very good.

When used as anodes under the conditions specified in Example 1 the plates thus coated showed an initial overvoltage of approximately 190 mV and then of 198 mV after the liberation of 55 tons of chlorine/m<sup>2</sup> of anodic surface at an anodic current density of 10 kA/m<sup>2</sup>. After production of 138 tons of chlorine/m<sup>2</sup>, the limit of useful life of the electrode had not yet been reached

and the consumption test was continued, but it was already apparent that the consumption of noble metal would be less than 41 mg/ton of chlorine produced.

Example 10 :  $ABO_4.4MO_2$  where A = Al, B = Ta and M = Ru

To 10 ml of the solution A of Example 1, there were added 1.25 ml of solution E of Example 3, 1.25 ml of the solution I of Example 9 and 37.5 ml of n-hexanol. The application of the composition, in 10 coats, to plates of etched titanium and the various heat treatments were carried out as in Example 1.

The average weight of the coatings thus obtained was approximately 6.8 g/m<sup>2</sup>; they contained 4 g-atom Ru to 1 g-atom Al and 1 g-atom Ta. The adherence to the substrate was very good.

When used as anodes under the conditions specified in Example 1 the plates thus coated showed an initial overvoltage of approximately 145 mV, at a current density of 10 kA/m<sup>2</sup>.

When submitted to the consumption test under the same conditions as in Example 1, the plates had produced more than 131 tons of chlorine/m<sup>2</sup> of anodic surface. At this time, the limit of useful life of the electrode had not yet been reached and the consumption test was continued, but it was already apparent that the consumption of noble metal would be less than 26 mg/ton of chlorine produced.

Example 11 :  $ABO_4.2MO_2$  where A = 0.9 Rh + 0.1 Yb, B = Sb and M = Ru

A solution J containing 1 g-atom Sb/liter was prepared by dissolving antimony pentachloride in isopropanol and a solution K containing 0.1 g-atom Yb/liter by attacking ytterbium oxide  $Yb_2O_3$  with hydrochloric acid and dissolving in isopropanol.

By mixing 10 ml of solution G of Example 9, 4.5 ml of solution H of Example 9, 2.5 ml of solution K, 2 ml of solution J and 30.5 ml of isopropanol, a coating composition was obtained, which was applied, in 10 coats, to plates of titanium etched under the same conditions as in Example 1. The various heat treatments were carried out by the same manner.

The average weight of the coatings thus obtained was approximately 8.0 g/m<sup>2</sup>; they contained 2 g-atom Ru to 0.9 g-atom Rh, 0.1 g-atom Yb and 1 g-atom Sb. The adherence to the substrate was excellent.

When used as anodes under the conditions specified in Example 1 the plates thus coated showed an initial overvoltage of approximately 122 mV at an anodic current density of 10 kA/m<sup>2</sup>.

When submitted to the consumption test under the same conditions as in Example 1, the plates had produced more than 103 tons of chlorine/m<sup>2</sup> of anodic surface. At this time, the limit of useful life of the electrode had not yet been reached and the consumption test was continued, but it was already apparent that the consumption of noble metal would be less than 41 mg/ton of chlorine produced.

The data of the illustrative Examples 1 to 11 are collected together in Table 1.

It will be understood that the above description of the present invention is susceptible to various modifications, changes and adaptations, and the same are intended to be comprehended within the meaning and range of equivalents of the appended claims.

TABLE 1.

| COMPILATION OF RESULTS ACHIEVED IN THE EXAMPLES. |                                                                           |                                 |                          |                                                    |                                                             |                                                                        |
|--------------------------------------------------|---------------------------------------------------------------------------|---------------------------------|--------------------------|----------------------------------------------------|-------------------------------------------------------------|------------------------------------------------------------------------|
| Example No.                                      | Coating composition                                                       | Wt. of coating g/m <sup>2</sup> | Adherence of the coating | Initial over-voltage in mV at 10 kA/m <sup>2</sup> | Consumption of Cl <sub>2</sub> produced in t/m <sup>2</sup> | test of the coating noble metal consumed mg/t Cl <sub>2</sub> produced |
| 1                                                | RhSbO <sub>4</sub> .2RuO <sub>2</sub>                                     | 4.5                             | excellent                | 165                                                | > 264                                                       | < 10                                                                   |
| 2                                                | RhNbO <sub>4</sub> .2RuO <sub>2</sub>                                     | 3.7                             | very good                | 245                                                | 81                                                          | 26                                                                     |
| 3                                                | AlSbO <sub>4</sub> .2RuO <sub>2</sub>                                     | 6                               | excellent                | 156                                                | 125                                                         | 20                                                                     |
| 4                                                | RhSbO <sub>4</sub> .2IrO <sub>2</sub>                                     | 6                               | excellent                | 200                                                | > 172                                                       | < 23                                                                   |
| 5                                                | RhSbO <sub>4</sub> 146 .4IrO <sub>2</sub>                                 | 3                               | excellent                | 230                                                | > 198                                                       | < 11                                                                   |
| 6                                                | RhSbO <sub>4</sub> .2(Ru <sub>2/3</sub> Ir <sub>1/3</sub> )O <sub>2</sub> | 7                               | excellent                | 135                                                | > 233                                                       | < 18                                                                   |
| 7                                                | RhSbO <sub>4</sub> .2(Ru <sub>1/3</sub> Ir <sub>2/3</sub> )O <sub>2</sub> | 6                               | excellent                | 135                                                | > 225                                                       | < 17                                                                   |
| 8                                                | RhSbO <sub>4</sub> .2RuO <sub>2</sub>                                     | 12                              | very good                | 112                                                | > 225                                                       | < 29                                                                   |
| 9                                                | RhTaO <sub>4</sub> .4RuO <sub>2</sub>                                     | 9.9                             | very good                | 190                                                | > 138                                                       | < 41                                                                   |
| 10                                               | AlTaO <sub>4</sub> .4RuO <sub>2</sub>                                     | 6.8                             | very good                | 145                                                | > 131                                                       | < 26                                                                   |
| 11                                               | (Rh <sub>0.9</sub> Yb <sub>0.1</sub> )SbO <sub>4</sub> .2RuO <sub>2</sub> | 8                               | very good                | 122                                                | > 103                                                       | < 41                                                                   |

We claim:

1. A metallic electrode for electrochemical processes comprising a metal support and on at least a portion of said support a conductive coating consisting essentially of a compound ABO<sub>4</sub> with a structure of the rutile-type, where A represents an element in the trivalent state selected from the group consisting of Rh, Al, and Ga and B represents an element in the pentavalent state selected from the group consisting of Sb, Nb and Ta, and an oxide of the type MO<sub>2</sub> where M is selected from the group consisting of Ru and Ir, and the mole ratio of ABO<sub>4</sub> to MO<sub>2</sub> is from 1/1 to 1/6.

2. A metallic electrode as claimed in claim 1, where A is an element in the trivalent state selected from the group consisting of Rh and Al.

3. A metallic electrode as claimed in claim 1, where B is pentavalent Sb.

4. A metallic electrode as claimed in claim 1 wherein the metal support is a valve metal.

5. A metallic electrode as claimed in claim 1 wherein the compound ABO<sub>4</sub> is RhSbO<sub>4</sub>.

\* \* \* \* \*

30

35

40

45

50

55

60

65